

[54] **PROCESS FOR INHIBITING FORMATION OF INTERMETALLIC COMPOUNDS IN CARBOTHERMICALLY PRODUCED METALS**

[75] Inventors: **Alex R. Valdo**, Elgin, Ill.; **Freeman M. Sanderford**, Dalton, Ga.

[73] Assignee: **Ethyl Corporation**, Richmond, Va.

[\*] Notice: The portion of the term of this patent subsequent to Oct. 26, 1988, has been disclaimed.

[22] Filed: **Sept. 11, 1972**

[21] Appl. No.: **287,974**

**Related U.S. Application Data**

[63] Continuation-in-part of Ser. No. 164,952, July 21, 1971, Pat. No. 3,704,117, which is a continuation-in-part of Ser. No. 744,307, July 12, 1968, Pat. No. 3,615,343.

[52] U.S. Cl. .... **75/68 A; 75/5 B; 264/12; 264/13**

[51] Int. Cl. .... **C22B 21/06**

[58] **Field of Search** .... **75/68 R, 68 A, 148, .5 B, 75/5 C, .5 R, .5 A; 148/11.5 A; 264/12, 13,**

[56] **References Cited**

**UNITED STATES PATENTS**

|           |         |                           |         |
|-----------|---------|---------------------------|---------|
| 2,738,548 | 3/1956  | Kassel .....              | 264/14  |
| 2,967,351 | 1/1961  | Roberts et al. ....       | 75/5 B  |
| 3,325,279 | 6/1967  | Lawrence et al. ....      | 75/148  |
| 3,374,089 | 3/1968  | Robinson, Jr. et al. .... | 75/68 R |
| 3,615,343 | 10/1971 | Valdo et al. ....         | 75/5 B  |
| 3,704,117 | 11/1972 | Valdo et al. ....         | 75/5 C  |

*Primary Examiner*—M. J. Andrews  
*Attorney, Agent, or Firm*—Donald L. Johnson; John F. Sieberth; Paul H. Leonard

[57] **ABSTRACT**

A process for inhibiting formation of intermetallic compounds in metal and metalloid containing alloys produced by carbothermic reduction of clay or ore, wherein molten alloy is removed from a reduction furnace, transferred to a holding pot, ladle or other suitable container, maintained at a temperature at least as high as the melting temperature of the lowest melting intermetallic compound, and then rapidly cooling the alloy, thereby minimizing the formation of intermetallic compounds. Cooling is preferably achieved by blowing the melt or by quenching.

**11 Claims, No Drawings**

**PROCESS FOR INHIBITING FORMATION OF  
INTERMETALLIC COMPOUNDS IN  
CARBOHERMATICALLY PRODUCED METALS**

**CROSS-REFERENCES TO RELATED  
APPLICATIONS**

This application is a continuation-in-part of U.S. application Ser. No. 164,952, filed July 21, 1971, now U.S. Pat. No. 3,704,117, which in turn is a continuation-in-part of U.S. application Ser. No. 744,307, filed July 12, 1968, now U.S. Pat. No. 3,615,343.

This invention is directed toward a novel technique for purification of alloys, and aluminum alloys in particular. Since many alloys contain undesirable impurities, it is frequently necessary to remove these impurities or at least reduce the quantity thereof before beneficial use can be made of the alloy. Consequently, there presently exists a need for a simple and inexpensive method for purifying alloys by reducing the quantity of undesirable impurities, such as intermetallic compounds, in these alloys.

This invention is particularly directed toward a process for purifying alloys produced by carbothermic reduction of clay or ore. Aluminum alloys manufactured by the carbothermic reduction technique frequently contain, in addition to free aluminum, varying quantities of aluminum, silicon, iron and titanium in various intermetallic forms. Considerable heat is necessary to carbothermically reduce a natural ore or clay to a metal alloy. Furnace temperatures of about 2000°C to about 2300°C are normally required to produce an aluminum-silicon alloy from an alumina-silica ore. The present invention provides a means for inhibiting the formation of these intermetallic compounds utilizing the heat produced in the carbothermic reduction process.

Accordingly, it is an object of this invention to provide a process for reducing the content of undesirable intermetallic compounds in various alloys produced by carbothermic reduction of clay by thermally causing the compounds to dissociate.

Another object of the invention is the purification of such carbothermically produced alloys which can be utilized commercially after removal of certain impurities.

In accordance with this invention, there is provided a process for reducing the content of one or more undesirable intermetallic compounds in a carbothermically produced alloy by transferring molten alloy directly from a carbothermic reduction furnace to a ladle or other suitable holding container and maintaining the molten alloy at a high enough temperature for a sufficiently long time to inhibit the formation of the intermetallic compounds and then rapidly cooling the alloy to minimize formation of the intermetallic compounds. The heat retained prevents formation of the intermetallic compound or compounds to the constituent elements and the subsequent quenching retards formation of these undesirable compounds by effecting a rapid temperature drop through the formation temperature of the compound.

The invention is characterized by convenient flexibility in that substantially any alloy containing one or more undesirable intermetallic compounds can be purified provided the alloy is capable of undergoing peritectic decomposition. The term "peritectic" may be

defined as an isothermal reversible reaction in which a molten liquid phase reacts with a solid phase to produce another solid phase on cooling. This invention is directed toward the elimination of, or at least reduction

5 in, the amount of certain intermetallic compounds present in this solid phase formed when the molten alloy is cooled. Thus, the term "peritectic decomposition" is used to denote the process of reducing the quantity of certain intermetallic compounds present in 10 the alloy. This is accomplished by transferring the molten alloy from the reduction furnace to a holding container and maintaining the alloy at a temperature above the formation temperature of the intermetallics then rapidly quenching the alloy by blowing the melt, with 15 ice water or in other suitable manner, to minimize the formation of the undesirable intermetallic compounds in the solid phase produced by cooling of the molten alloy. In this manner it has been found that a solid phase may be formed which contains innocuous amounts of the compound sought to be eliminated.

Substantially any alloy may be easily purified according to the techniques of this invention, magnesium alloys, zinc alloys and the like being exemplary. Alloys containing aluminum are particularly well suited to upgrading by the instant process. Aluminum alloys which are readily susceptible to purification may have an aluminum content varying from a fraction of a percent up to 99 percent and higher.

30 Aluminum alloys which are particularly susceptible to purification by this process are those containing from about 40% to about 90% aluminum by weight. The aluminum may be alloyed with substantially any element so long as one or more intermetallic compounds are present, the removal of which is desired.

35 Exemplary of the metals and metalloids which may be present as intermetallics with aluminum in these alloys are iron, carbon, silver, boron, calcium, cobalt, chromium, manganese, nickel, titanium, uranium, vanadium, zinc, copper and silicon. Two or more of these, 40 and other elements may be present in varying proportions with aluminum and may easily be removed from the alloy by the process of this invention. For example, common aluminum alloy-intermetallic constituents which readily undergo peritectic decomposition and which are therefore susceptible of being removed by application of the inventive process are  $FeAl_3$ ,  $MnAl_6$ ,  $CuMgAl_2$ ,  $TiAl_3$ ,  $FeSi_2Al_4$  and  $Al_2Ti_5Si_8$ .

50 Of the foregoing intermetallic compounds which are frequently found to be undesirable constituents of aluminum alloys, compounds containing at least 2 of the elements, aluminum, silicon, titanium, iron, copper, magnesium and manganese are particularly significant because they are frequently found in those alloys obtained by the carbothermic reduction of clay.

55 Common intermetallic compounds contained in carbothermically produced aluminum alloys are  $FeSi_2Al_4$  and  $TiAl_3$ . It will be recognized that many other combinations are frequently found. It has been found that by application of this invention such undesirable intermetallic compounds may be thermally decomposed, thereby enriching the aluminum content of the base aluminum alloy.

60 As previously noted, a basic feature of the invention is retaining sufficient heat in the impure alloy to maintain its temperature at least above the melting point of the intermetallic compound which is to be inhibited from forming in the alloy. Suitable temperatures which

may be utilized in the invention are dependent upon the melting temperature of the intermetallic compound which is to be reduced in any given alloy. In general, however, temperatures in the range of from about 300°C to about 1400°C are high enough to melt intermetallic compounds which are susceptible to peritectic decomposition. For example, if decomposition of the intermetallic  $\text{FeSi}_2\text{Al}_4$  is to be accomplished in an aluminum alloy containing by weight about 68% aluminum, 27% silicon, 3% iron and 2% titanium, the alloy should be maintained at a temperature of at least 870°C (which is the melting temperature of this intermetallic compound) before rapid cooling is effected. Similarly, if it is desirable to remove  $\text{TiAl}_3$  from an alloy having the same or a similar composition, a temperature of at least 1340°C should be maintained before quenching the alloy.

In order to insure that substantially all of the intermetallic compound is melted, it is preferable to keep sufficient heat in the alloy to maintain the alloy at a temperature somewhat above the melting point of the intermetallic, sufficiently above the melting point to yield a fluid melt. In blowing from the melt, the alloy containing the intermetallics must be maintained at a temperature sufficiently high to keep the metal molten. The metal must be in a fluid state before it can be blown.

The length of time at which the alloy should remain at the intermetallic melting point is not critical, but it should be long enough to insure that all of the undesirable intermetallic compound or compounds are maintained in a molten state.

After the molten alloy is tapped from the furnace and transferred to a holding pot or ladle, it should be maintained at an appropriate temperature to prevent formation of the intermetallic compounds. When solidification of the alloy is desirable, it should be rapidly cooled in order to prevent the formation of these compounds, as heretofore noted. Rapid cooling is accomplished by blowing the melt, or quenching, the procedures for which are described hereinafter.

The equipment satisfactory for carrying out the blowing of a molten alloy consists of a graphite crucible equipped with an induction heating coil wrapped around the outside of the crucible so that the charge can be heated to the desired temperature by induction. The crucible has a hole in the bottom thereof to which is attached a graphite tube. A graphite rod is placed in the crucible to close the graphite tube and contain the molten alloy in the crucible until the blowing operation is conducted. Twenty-four air jets are mounted concentrically around the graphite tube in the shape of a cone with the apex of the cone pointed downward so that the stream of air which is discharged from the jets is directed to the discharge end of the graphite tube. This assembly is mounted on a refractory slab which in turn mounted on a metal cylinder. The graphite tube and air jets extend through a hold in the refractory cover so that the blown powder is retained by and collected in the metal cylinder. The metal cylinder is equipped with openings at its top to serve as vents for the air discharged through the air jets.

The alloy to be treated is charged in molten form to the graphite crucible. The crucible is heated by induction to the desired temperature to maintain a homogeneous, fluid melt of alloy. The induction field induces a gentle rolling action within the melt which maintains homogenization.

After a desired time, a valve is opened to admit air to the jets mounted around the bottom of the graphite tube. The graphite rod is then removed from the crucible, and the molten alloy flows through the graphite tube and is atomized by the air from the jets. The atomized alloy falls downward in the metal cylinder, cools and solidifies and is collected in the bottom of the cylinder. If the metal cylinder is tall enough, the alloy will be cooled sufficiently by the flow of air. If it is not practical to use a tall cylinder, a pool of water can be placed in the bottom of the metal cylinder to effect final cooling and solidification.

The particle size of the blown power can be controlled by varying the air pressure applied to the air jets and/or the diameter of the tube through which the molten alloy is discharged from the crucible. In general, the higher the air pressure, the smaller the particle size of the product alloy; the smaller the tube diameter, the smaller the particle size. However, the tube diameter cannot be so small that the molten alloy cools and solidifies in the tube. In general, the finer the particle size the more rapid is the cooling of the molten alloy and the less is the likelihood of undesirable intermetallics in the final product.

This apparatus has been used by others to prepare pure metal powders and alloys. For example, nickel powder has been prepared by personnel in the Canadian Department of Mines using an apparatus and melt blowing procedure similar to the foregoing.

Variations of the above apparatus and procedure can be employed with equal effectiveness. Hence, instead of having the air jets impinging on the stream of molten metal to atomize the molten metal, the air can be introduced into the tube above its discharge end and the alloy forced through a nozzle attached to the end of the tube to atomize the molten metal. Gases other than air such as argon and nitrogen may be used provided they do not react with and contaminate the alloy to any great extent. A stream of water may be used in place of air, and the use of argon instead of air is especially suitable when it is desired to produce an alloy powder having a minimum oxygen content. Materials of construction may be used other than graphite, the main requirement being that they are compatible with the molten alloy.

Generally, a smaller residue of the undesirable intermetallic compound has been found in the alloy subjected to melt blowing as compared to an alloy of the same composition which has been subjected to other quenching techniques.

Another method for rapidly cooling the molten alloy is the use of an ice water quench to lower the temperature of the molten alloy as rapidly as possible. Of course, it will be recognized by those skilled in the art that many other quenching media and techniques may be utilized successfully in the cooling phase of this invention. In general, it is preferably to quench the alloy at a rate of from about 100° to about 400° per second, and most preferably, about 200° per second.

It has been found that the product alloy, that is, the alloy which has been purified by the technique of this invention, may be best commercially utilized in small particles. Of course, size reduction of the purified alloy may be undertaken after purification by conventional techniques such as crushing, grinding, and other methods well known to those skilled in the art. However, size reduction may be easily effected in the course of

this process by sieving the molten alloy after heating it to the appropriate temperature. Thus, the molten alloy may be poured through a screen having a mesh size proportional to the size of the finished alloy particle desired, and when it is desired to utilize a liquid quench for cooling purposes, the molten alloy may be poured through a screen or similar size reducing apparatus directly into the quenching medium.

Accordingly, a preferred embodiment of the invention is characterized by utilizing a molten alloy prepared by carbothermic reduction, containing aluminum, silicon, iron and titanium, wherein the intermetallic compounds usually formed are composed of aluminum, silicon and iron and aluminum and titanium, respectively, maintaining a temperature within the range of from about 300°C to about 1400°C and then rapidly cooling the molten alloy by rapidly blowing the melt. In a more preferred embodiment, the alloy contains by weight about 68% aluminum, 27% silicon, 3% iron and 2% titanium, the usually formed intermetallic compounds are  $FeSi_2Al_3$ , the molten alloy is maintained in an inert atmosphere at a temperature of about 1340°C or higher keeping the melt fluid, after which the alloy is cooled by rapidly blowing the melt, quenching or the like.

As heretofore mentioned, it is desirable to inhibit formation of certain undesirable intermetallic compounds normally present in alloys without simultaneously producing additional undesirable compounds. Consequently, the inventive process defines a technique for inhibiting the formation of intermetallic compounds in a variety of metal and metalloid-containing alloys produced by carbothermic reduction transferring the molten alloy to a suitable container and maintaining the alloy at a temperature at least as high as the melting temperature of the intermetallic compound to be prevented from forming but below the melting temperature of at least one of the metals or metalloids in the alloy, the yield of which it is desired to increase. Once solidification of the alloy is desired, the alloy should be rapidly cooled by blowing the melt, quenching or the like.

This technique prevents the formation of undesirable intermetallics in the alloy. Subsequent rapid cooling of the alloy substantially preserves the elemental components and inhibits formation of the undesirable intermetallics and minimizes the formation of other undesirable compounds containing the metal or metalloid. In this aspect of the invention a preferred alloy is composed of aluminum, silicon, iron and titanium.

In one embodiment of the invention where the alloy contains the metalloid, silicon, it is desirable to maintain the alloy at a temperature above the melting point of the intermetallic compound or compounds to be decomposed but below the melting temperature of the silicon, and then rapidly cool the alloy in order to increase the yield of silicon in the cooled alloy. As above noted, this technique inhibits formation of intermetallic compounds in the alloy and also substantially reduces the amount of silicon-containing compound in the quenched alloy. In this manner, the quantity of elemental silicon or other element in a given alloy may be increased. As in previous embodiments of the invention, the temperature may generally be maintained within the range of from about 300°C to about 1400°C and should be maintained sufficiently high to maintain the melt in molten condition. Further, the cooling stage of

the process is effected by rapidly blowing the melt, quenching or the like.

In a most preferred embodiment of the invention the alloy treated contains by weight about 68% aluminum, 27% silicon, 3% iron and 2% titanium and the intermetallic compounds tending to be formed are  $FeSi_2Al_4$ ,  $Al_2Ti_3Si_8$  and  $TiAl_3$ . Further, the molten alloy is maintained at a temperature of about 1340°C (which is below the melting point of silicon) in an inert atmosphere such as nitrogen or argon. The cooling phase is effected by rapidly blowing the melt.

This invention and the various embodiments thereof may be further understood by the following illustrative examples. In all cases the alloy used was a synthetic alloy which simulated an alloy produced by a carbothermic reduction process.

#### EXAMPLE I

Approximately 500 grams of an alloy containing by weight 68 percent aluminum, 27 percent silicon, 3 percent iron and 2 percent titanium and having a  $FeSi_2Al_4$  content of about 20 weight percent were heated to 1,000°C in a large crucible and held at this temperature for 30 minutes. The molten metal was then rapidly quenched in ice water by pouring the alloy directly into a water-ice mixture having a temperature of 2°C. After the quenching operation, the alloy was analyzed and found to contain 5.5 percent by weight of the  $FeSi_2Al_4$  intermetallic compound.

#### EXAMPLE II

Three hundred forty-five grams of an alloy having the same composition as that used in Example II were heated in a crucible to a temperature of 1,000°C where it was held for 15 minutes and vigorously stirred. The molten alloy was then poured through a stainless steel screen into ice water, the temperature of which was 2°C. Small particles of alloy were observed to form in the ice water. The analysis of  $FeSi_2Al_4$  present in the alloy after quenching was found to be 9 percent by weight.

#### EXAMPLE III

Ten grams of silicon alloy containing 75 percent by weight of silicon, 5 percent by weight of aluminum, 19 percent by weight of  $FeSi_2Al_4$  and 1 percent by weight of  $TiAl_3$  were heated in a crucible to 1200°C and held at that temperature for 15 minutes. The alloy was then allowed to cool in air. The cooled alloy was subjected to X-ray analysis which showed on a weight basis, 82.4 percent silicon, 1.6 percent aluminum, 7.4 percent  $FeSi_2Al_4$  and the presence of two unknown intermetallic compounds.

#### EXAMPLE IV

Twenty-five grams of an alloy containing by weight 73 percent silicon, 5 percent aluminum, 22 percent  $FeSi_2Al_4$  and a trace of  $TiAl_3$  were heated in an argon atmosphere to 1,000°C, held for 15 minutes and subsequently quenched in ice water. Upon X-ray analysis, the  $FeSi_2Al_4$  content was found to be 2.2 percent by weight and there appeared to be no trace of  $TiAl_3$  left in the alloy.

#### EXAMPLE V

Three 10 gram samples of aluminum alloy containing by weight 27.4 percent aluminum, 50.2 percent silicon,

8 percent iron ( $FeSi_2Al_4$ ) was present in an amount equal to 19 percent by weight) and 0.4 percent titanium were heated to temperatures of 800°C, 900°C and 1000°C, respectively. The alloy samples were held at these respective temperatures for 15 minutes and were then rapidly quenched in ice water. X-ray analysis of the three samples showed the  $FeSi_2Al_4$  content of the samples by weight as follows: 800°C - 14.9 percent; 900°C - 14.9 percent; 1000°C - 1.9 percent.

Example V clearly illustrates that for best results the alloy to be purified should be heated to a temperature significantly above the melting point of the intermetallic compound to be decomposed. The melting point of  $FeSi_2Al_4$ , as previously noted, is about 870°C, and the results of Example V show that much more  $FeSi_2Al_4$  impurity is removed by quenching from a temperature of 1000°C (well above 870°C) than from the temperatures below and even slightly above the intermetallic compound melting point.

From an analysis of the preceding examples and embodiments it is apparent that the invention provides an easy and economical method for decomposing a quantity of undesirable intermetallic compound in virtually any alloy capable of undergoing peritectic decomposition. Operation procedures are simple and necessary equipment is not expensive and is readily available. Accordingly, the invention contributes to the art of alloy purification.

#### EXAMPLE VI

A sample of Al-Si-Fe-Ti alloy, having the composition by weight 62% Al, 33% Si, 2% Fe, 3% Ti, was melted at 1250°C to give a homogeneous liquid which was then atomized by allowing it to flow through a  $\frac{1}{4}$  inch tube and directing a stream of water at 200 psi onto the molten metal stream. The resultant powder was 95% - 30 mesh and 85% 100 + mesh. X-ray diffraction analysis of the resultant powder gave a diffraction pattern which contained no peaks assignable to the  $FeSi_2Al_4$  intermetallic and only two small peaks which might be assignable to an Al-Si-Ti intermetallic. Hence, the product contained at most trace amounts of the Al-Si-Ti intermetallic. On the other hand, a comparison sample having essentially the same composition but which was cooled and crystallized slowly gave an X-ray pattern which showed the presence of small, but detectable amounts of  $FeSi_2Al_4$  and about 6% of the Al-Si-Ti intermetallic.

#### EXAMPLE VII

An aluminum-silicon-iron-titanium alloy composition was prepared by placing weighed amounts of the individual metals in a graphite crucible and heating the crucible in an induction coil to 1400°C to form a fluid homogeneous melt which was held at 1400°C for 15 minutes. The molten alloy was then forced through a discharge tube under argon pressure and atomized by blowing the metal through a nozzle connected to the end of the discharge tube. The blown alloy was analyzed by X-ray fluorescence (XRF). X-ray diffraction (XRD) analysis of the powder showed it to contain little or no intermetallics as set forth in Table I hereinafter.

Two other Al-Si-Fe-Ti alloy compositions were prepared by melting weighed amounts of the individual metals in a graphite crucible. However, these samples were not blown from the melt. Instead, the crucible and

molten alloy were removed from the furnace and allowed to cool to room temperature. The solid alloy samples were removed from the crucibles, crushed and ground. X-ray fluorescence (XRF) and X-ray diffraction (XRD) analyses of these samples are also set forth in Table I.

TABLE I

| Sample No. | Alloy Compositions |      |     |     |
|------------|--------------------|------|-----|-----|
|            | Al                 | Si   | Fe  | Ti  |
| 1          | 62.2               | 33.3 | 1.4 | 1.0 |
| 2A         | 61.9               | 33.6 | 1.3 | 1.4 |
| 2B         | 59.5               | 31.7 | 1.8 | 1.5 |

  

| Sample No. | Percent Intermetallics in Alloy (XRD) |                |          |
|------------|---------------------------------------|----------------|----------|
|            | $FeSi_2Al_4$                          | $Al_2Ti_5Si_8$ | $Fe_2Ti$ |
| 1          | None                                  | 1              | None     |
| 2A         | Trace                                 | 3              | 1        |
| 2B         | 2                                     | 4              | Trace    |

It can be clearly seen that both cast and ground samples (2A and 2B) contained more intermetallics than did the sample (1) blown from the melt.

#### EXAMPLE VIII

An alloy composition was prepared and blown according to the procedure of Example II. The composition of the resultant powder was determined by X-ray fluorescence to be 56.0% Al, 32.7% Si, 3.1% Fe and 2.8% Ti. X-ray diffraction analysis detected 2%  $FeSi_2Al_4$  and 5%  $Al_2Ti_5Si_8$ ; no  $Fe_2Ti$  was detected.

For comparison, a second alloy sample was prepared, but was cooled, crushed and ground (instead of being blown). Its composition was determined by X-ray fluorescence to be 55.2% Al, 28.5% Si, 3.4% Fe and 2.8% Ti. It was found to contain by X-ray diffraction 3%  $FeSi_2Al_4$ , 7%  $Al_2Ti_5Si_8$  and about 1%  $Fe_2Ti$ .

Again, it has been clearly demonstrated that substantially less intermetallics are found when the alloy has been rapidly cooled by blowing the melt.

From an analysis of the preceding examples and embodiments it is apparent that the invention provides an easy and economical method for inhibiting the formation of undesirable intermetallic compound in virtually any carbothermically produced alloy capable of undergoing peritectic decomposition. Operating procedures are simple and necessary equipment is inexpensive and is readily available. Accordingly, the invention contributes to the art of alloy purification.

The foregoing disclosure and description of the invention is illustrative and explanatory thereof and various changes may be made within the scope of the appended claims without departing from the spirit of the invention.

What is claimed is:

1. In a process comprising carbothermically reducing an ore to form a molten alloy, the improvement in combination therewith for inhibiting the formation of intermetallic compounds in metal and metalloid-containing alloys produced by the carbothermic reduction of the ore and capable of undergoing peritectic decomposition, comprising the steps of transferring the molten carbothermically produced alloy from a carbothermic reduction furnace to a suitable container, maintaining the transferred alloy in the container at a temperature at least as high as the melting temperature of any undesirable intermetallic compound but below the melting

temperature of at least one of the metals or metalloids in the alloy, the yield of which it is desired to increase, and then rapidly cooling the alloy, thereby minimizing the formation of an undesirable intermetallic compound.

2. The process of claim 1, wherein the molten alloy is an aluminum alloy.

3. The process of claim 1, wherein said molten alloy contains aluminum, silicon, iron and titanium.

4. The process of claim 1, wherein at least one of the 10 metals is silicon.

5. The process of claim 1, wherein said molten alloy is maintained at a temperature within the range of from about 300°C to about 1400°C and sufficiently high to maintain the alloy in a molten state.

6. The process of claim 1, wherein said rapid cooling is effected by rapidly contacting the alloy with a quenching medium.

7. The process of claim 1, wherein said rapid cooling is effected by blowing the melt.

8. The process of claim 1, wherein the molten alloy is sieved after being transferred from the carbothermic reduction furnace.

9. The process of claim 1, wherein (a) the molten alloy contains by weight about 68 percent aluminum, 27 percent silicon, 3 percent iron and 2 percent titanium; (b) the molten alloy is maintained in an inert atmosphere at a temperature of about 1340°; and (c) said subsequent rapid cooling is effected by rapidly contacting the alloy with ice water.

15 10. The process of claim 9, wherein the alloy is sieved before being contacted with said ice water.

11. The process of claim 9, wherein said rapid cooling is effected by rapidly blowing the melt.

\* \* \* \* \*

20

25

30

35

40

45

50

55

60

65

UNITED STATES PATENT OFFICE  
CERTIFICATE OF CORRECTION

PATENT NO. : 3,910,787

DATED : October 7, 1975

INVENTOR(S) : A. R. Valdo and F. M. Sanderford

It is certified that error appears in the above-identified patent and that said Letters Patent are hereby corrected as shown below:

Column 3, lines 56 and 57, "which in turn mounted" should read -- which in turn is mounted -- . Column 4, line 13, "power" should read -- powder -- . Column 4, line 58, "preferably" should read -- preferable -- . Column 5, line 21, "FeSi<sub>2</sub>Al<sub>3</sub>" should read -- FeSi<sub>2</sub>Al<sub>4</sub> and TiAl<sub>3</sub> -- . Column 6, line 33, "Example II" should read -- Example I -- .

Signed and Sealed this  
sixth Day of January 1976

[SEAL]

Attest:

RUTH C. MASON  
Attesting Officer

C. MARSHALL DANN  
Commissioner of Patents and Trademarks